

## UNITED STATES PATENT OFFICE.

RALPH P. DE VRIES, OF MENANDS, AND HENRY A. DE FRIES, OF ALBANY, NEW YORK,  
ASSIGNORS TO LUDLUM STEEL COMPANY, OF WATERVLIET, NEW YORK, A COR-  
PORATION OF NEW JERSEY.

## STABLE-SURFACE ALLOY STEEL RESISTANT TO ACIDS.

No Drawing.

Application filed November 26, 1926. Serial No. 151,013.

This invention relates to alloys of steel and more particularly to such alloys which are commonly designated as stable surface acid resistant steels.

5 The main objects of our invention are to provide an alloy steel of new composition which will be resistant to sulphuric acid in all percentages of dilution, whether the acid be used in the cold or in the hot condition, and 10 which will further be resistant to mixtures of sulphuric and nitric and to certain dilutions of hydrochloric acid.

The invention is of particular utility for 15 steel tanks, valves, and fittings of various kinds which are used where they come into contact with acids such as are employed in commercial or manufacturing operations, and finds particular application where steel is required for strength and is at the same 20 time exposed to sulphuric acid diluted to any degree.

The alloy steel of our invention contains nickel from 14% to 30%, chromium from 6% to 20%, silicon from 1% to 3%, tantalum 25 from 1% to 3%, carbon from as low as possible content up to 1%. Manganese may be present in amounts usually found in alloy steels, up to .75%, and the usual amounts of metalloids, such as phosphorus and sulphur 30 may be present. The carbon content varies in all cases with the amount of nickel, and their approximate relative proportions are expressed by the equation  $x=1.6-0.06y$ , where  $x$  is the carbon content in per cent and  $y$  the 35 nickel content in per cent.

We do not wish to be held exactly to the equation just given, but as near as we can determine it sets forth the limiting condition between the carbon and nickel content.

40 For best results, we have found that the silicon and the tantalum must always be used in approximately equal quantities; that is, if silicon is used in the amount of 1-1/2%, it is desired to have tantalum in a nearly similar 45 amount.

As already stated, alloy steels made within this range of composition are particularly resistant to the action of sulphuric acid, whether the acid is used cold or hot.

50 The following is a good example of a pre-

ferred analysis which we wish to make in this range:

|           | Per cent. |
|-----------|-----------|
| Carbon    | 0.45      |
| Manganese | 0.50      |
| Nickel    | 18.00     |
| Chromium  | 10.00     |
| Silicon   | 2.00      |
| Tantalum  | 2.00      |

The attack which occurs is most pronounced 60 during the first 24 hours. Thereupon the material becomes extremely passive and corrosion proceeds at a uniform, but almost negligible rate. The protecting film formed during the first exposure of approximately 24 65 hours is of such a nature that it prevents, to all intents and purposes, further corrosion. It is important to note that the protecting film does not alternately break down and rebuild with consequent loss of the acid resist- 70 ant alloy steel.

The steel after attaining passivity is in a state of equilibrium with regard to acid attack, even if the degree of acid dilution is 75 changed frequently; that is, the tank containing acid might be washed out with water and the passivity of the steel previously set up through acid attack would not be broken down.

The corrosion tests against sulphuric acid 80 attack have shown that the loss in weight in all dilute sulphuric acid solutions below 20% is about equal. When the strength of the acid is increased from 20% to 40%, the attack on the alloy steel diminishes and after 85 the strength of the acid solution is increased from 50% to 100%, the attack is again slightly increased, being equal in the latter case to the losses in the dilute acids below 20%. The acid attack, no matter what the dilution 90 or condition of the acid, is so small in amount as to be practically negligible for most commercial purposes of which we have any knowledge.

The corrosion resistance of our alloy steel 95 against mixed acids, for instance, as sulphuric and nitric, is approximately as good as against sulphuric acid of different solutions.

In contra-distinction to most materials of 100

which we have any knowledge as being good acid resisting materials, the steel of our invention is easily melted; is malleable hot and to some extent cold and can be annealed so as to be easily machined. It can be melted in an electric furnace or otherwise; it can be cast in ingots and readily rolled into bars, shapes, or sheets as may be required. It casts with a good surface and can be cast into any form or shape desired, such castings can be annealed by heating from 1400° to 1600° F. and slowly cooled and when so annealed can be easily machined. Rolled and forged products can be annealed with similar results.

The physical properties of this material are good. The alloy steel having the tensile strength of about 85,000 pounds in the annealed condition and good impact shock resistance. These properties can be modified by heat treatment.

Essentially, the steel is not, however, a steel which can attain tool steel hardness. By air cooling after heating to 2100°, it will be possible to get a hardness of about 400 Brinnell which will be hard enough for many parts that must be hardened to resist wear; while at the same time resisting the attack of acids and acid fumes.

The alloy steel of our invention need not be cleaned of the hot scale of rolling or hammering or casting to make it resistant to the acid attack. The scale that is formed is very smooth and adherent. For many purposes it will be desirable to remove this scale and this may be done by the ordinary processes of machining and grinding. The clean metallic surface thus obtained will be equally resistant to acid attack.

The thermal coefficient of expansion of 40 this alloy steel is extremely low, which fact is useful where the distortion of working parts, due to temperatures obtained in a hot acid or acid fumes, must be controlled.

We have already described the passivity 45 that is set up after the first acid attack and have further noted that the state of equilibrium having once been reached by the alloy steel, is not again broken down.

We find that the additions of tantalum are 50 peculiarly effective in the alloy steel of our invention to maintain the passivity of the steel against acid attack once this has been established.

We claim:

1. As a new product, an alloy steel resistant to sulphuric and mixed acids, comprising nickel from 14% to 30%, chromium from 6% to 20%, silicon from 1% to 3%, tantalum from 1% to 3%, carbon from 0% to 1% 60 and the balance iron.

2. An alloy steel resistant to sulphuric and mixed acids, comprising nickel from 14% to 30%, chromium from 6% to 20%, silicon from 1% to 3%, tantalum from 1% to 3%, carbon in all percentages of the nickel range being substantially in accordance with the equation  $x=1.6-0.06y$ , where  $x$  is the carbon and  $y$  the nickel content. 65

3. An alloy steel resistant to sulfuric acid, 70 comprising nickel from 14% to 30%, chromium from 6% to 20%, silicon from 1% to 3%, tantalum from 1% to 3%, carbon from 0% to 1%, and the balance iron, the lesser amounts of carbon being used with the greater 75 amounts of nickel.

RALPH P. DE VRIES.  
HENRY A. DE FRIES.